

## UNITED STATES PATENT OFFICE

2,162,460

## VISCOSE-CELLULOSE ETHER SOLUTION

Robert W. Maxwell, Wilmington, Del., assignor to  
 E. I. du Pont de Nemours & Company, Wil-  
 mington, Del., a corporation of Delaware

No Drawing. Application January 8, 1938,  
 Serial No. 183,944

10 Claims. (Cl. 260—226)

This invention relates to regenerated cellulose (rayon), and more particularly to a regenerated cellulose which is superior to the heretofore known regenerated celluloses in dyeing properties 5 deformation properties, and moisture-proof film-retaining properties.

Ordinary regenerated cellulose film, which has been coated with a wax composition to render it moisture-proof, rapidly (in an hour or two) 10 loses its effectiveness in the presence of water. The loosening and detachment of the wax composition layer which results from contact with water precludes the use of such a material in many fields. Numerous efforts to overcome this 15 property of the regenerated cellulose have been made. These included, inter alia, the use of other (than wax) coating compositions and the use of intermediate films to anchor the wax coat to the regenerated cellulose, which would 20 increase undesirably the cost of the material.

It is also known that regenerated cellulose threads (filaments) reflect with a sort of magnifying effect small variations in regenerating conditions in such a way that large variations in 25 dyeing characteristics result. In addition, regenerated cellulose yarns do not dye as well as is desired with certain types of dyes, for example, direct dyes. This disadvantage (apparently a lack of affinity for important classes of dyes) has 30 been the incentive for much research, but up to the present time neither of these undesirable properties has been satisfactorily overcome.

It is also known that regenerated cellulose filaments and films possess the undesirable property 35 of expanding and contracting considerably with changes in humidity. This disadvantage has been a source of worry to the manufacturers and users of cellulose films, and has handicapped them for many years. Much time and money 40 have been spent in efforts to produce a regenerated cellulose film devoid of this drawback.

This invention had for an object the preparation 45 of a regenerated cellulose having superior dyeing characteristics. Other objects were the preparation of a regenerated cellulose having superior adherence to moisture-proof coatings, having improved resistance to deformation and having both good wet strength and desirable dyeing properties. Still further objects were the preparation 50 of new and improved viscose and regenerating procedures and products. A general advance in the art and other objects which will appear hereinafter are also contemplated.

It has now been found that all the aforementioned 55 obstacles to the use of regenerated cellulose

lose can be overcome by the simple expedient of incorporating in the viscose prior to regeneration a minor proportion of a low substituted cellulose ether which is soluble in dilute aqueous caustic soda. The resulting modified regenerated cellulose does not have the disadvantages described above. 5

It has previously been proposed that equal parts of viscose and caustic alkali solutions of cellulose ethers be spun into fibers. There seems to be 10 no particular advantage in such a process. Such mixtures give coagulated products having a wet strength too low to be spun by prevailing commercial methods. Even, when in order to get threads for experimental purposes, commercially 15 impractical procedures are employed, it is almost impossible to spin and handle the filaments because they stick together on the bobbin. In addition, the dried filaments of such mixtures are harsh and unpleasant to touch. 20

From the following description and specific examples, in which are disclosed certain embodiments of the invention as well as details of what is believed to be the best mode for carrying out the invention, it will be apparent how the foregoing objects and related ends are accomplished. 25 The quantities are given in parts by weight throughout the application.

## Example I

Twenty-five (25) parts of a 6% solution of a water soluble glycol cellulose in 7% aqueous caustic soda prepared as described in Example XXII, were mixed with 75 parts of a viscose containing 6% cellulose and 6% sodium hydroxide. 30 After ripening for 48 hours at 25° C. the mixture was cast into a transparent film in the usual way, and after drying, was coated with a moisture-proofing lacquer such as that described in United States Patent 1,737,187 issued November 26, 1929, to Charch. It was necessary to soak the 35 coated film in water at 25° C. for six days before the lacquer coating could be detached by rubbing gently between the fingers. 40

A film of regenerated cellulose prepared from 45 the same viscose in the same manner and coated with the same composition in the same manner could be separated from its lacquer coating with the same treatment after soaking in water at 25° C. for about two hours.

The glycol cellulose contained about one glycol 50 group per glucose unit of the cellulose. As a result the average composition of the cellulose-glycol cellulose mixture was one glycol group for every four glucose units present (i. e., both in 55

the cellulose and in the glycol cellulose). The films of the cellulose-glycol cellulose mixture were very much stronger when wet than films of glycol cellulose containing .25 glycol groups per glucose unit which had been coagulated from an alkali solution of the glycol cellulose. They were also very much stronger when wet than films of glycol cellulose containing .25 glycol groups per glucose unit which had been regenerated from a viscose-like solution of a xanthated glycol cellulose.

#### Example II

Five (5) parts of a 6% solution of a water soluble glycol cellulose in 7% aqueous caustic soda prepared as described in Example XXII were mixed with 95 parts of viscose containing 7% cellulose and 6% sodium hydroxide. After suitable ripening the mixture was cast into films in a sulfuric acid sodium sulfate bath by spreading a thin film on a glass plate and dipping it into the warm precipitating bath. The films were washed acid free with water, steeped in a 4% aqueous solution of glycerin and dried. The film after drying was coated with a moisture-proofing lacquer having a nitrocellulose base. After soaking in water at 25° C. for two days the moisture-proofing layer was still tightly bound to the base.

This product (moisture-proofed) has, after extensive tests, been found particularly suitable for milk bottle hoods.

The ratio of wet to dry strength of filaments made from the cellulose-glycol cellulose solution of this example was substantially the same as that of filaments made from the same viscose to which no glycol cellulose solution had been added, namely, 0.474. The average number of glycol groups present per glucose unit of cellulose plus glycol cellulose was 0.05. Filaments regenerated from a xanthated glycol cellulose containing 0.06 glycol groups per glucose unit had a ratio of wet to dry strength which was 0.396.

The aforementioned cellulose-glycol cellulose filaments showed a considerably greater affinity for Pontamine Sky Blue 6 BX (a direct dye, C. I. 518) than the aforementioned regenerated cellulose filaments.

#### Example III

One (1) part of a 6% solution of a water soluble glycol cellulose in 7% aqueous caustic soda prepared as described in Example XXII was mixed with 99 parts of viscose containing 7% cellulose and 6% sodium hydroxide. After suitable ripening the mixture was cast into films. These showed a markedly increased affinity for substantive dyestuffs compared with films made from the same viscose without modification.

#### Example IV

Ten (10) parts of a 7% solution in water of a water soluble sodium cellulose glycolate (containing 0.5 glycolic acid ether group per glucose unit of the cellulose) were mixed with 90 parts of a viscose solution containing 7% cellulose and 6% sodium hydroxide. The resulting solution was cast into films in the usual way and was then coated with a moisture-proofing lacquer. It was necessary to soak the resulting film in water for two days before the lacquer coating could be detached by rubbing gently with the fingers.

The wet strength of filaments prepared by the xanthation and regeneration of a cellulose glycolic acid containing the same average content of glycolic acid radicals as the cellulose-cellulose glycolic acid mixture was more than 10% lower.

The cellulose-cellulose glycolic acid mixture filaments had an increased affinity for basic dyes when compared with filaments from the same viscose which had not been modified.

#### Example V

Twenty-five (25) parts of a 7% solution in water of a water soluble sodium cellulose glycolate (containing 0.5 glycolic acid ether groups per glucose unit of the cellulose) were mixed with 75 parts of a viscose solution containing 7% cellulose and 6% sodium hydroxide. The resulting solution was cast into films. After moisture-proofing in the same way as that described in Example IV, a product was obtained which could be kept covered with water at ordinary normal room temperature for four days before it could be easily separated into base and moisture-proofing layers.

#### Example VI

Twenty-five (25) parts of a 7% solution of a water insoluble room temperature alkali-soluble glycol cellulose in 7% aqueous caustic soda described in Example XXIII were mixed with 75 parts of a viscose containing 7% cellulose and 6% sodium hydroxide. The resulting solution was ripened and cast into films. After moisture-proofing with a composition based on nitrocellulose, a product was obtained which exhibited a marked resistance to separation of the base layer and lacquer coating when immersed in water.

Filaments of the product spun at low tensions were found to possess a wet strength equivalent to about 80% of filaments spun from the same viscose under the same conditions, whereas filaments regenerated from a xanthated glycol cellulose of approximately the same average degree of substitution (0.18 mol of glycol radical per glucose unit) under corresponding conditions possessed a wet strength of only 50% of that of the viscose filaments.

#### Example VII

Two (2) parts of a 7% solution of a water insoluble room temperature alkali-soluble glycol cellulose in 7% aqueous caustic soda described in Example XXIII were mixed with 98 parts of a viscose containing 7% cellulose and 6% sodium hydroxide. The resulting solution was spun into filaments using a sulfuric acid bath of greater than 40% sulfuric acid strength. The resulting filaments possessed a wet strength substantially equivalent to that of filaments prepared in the same manner from the same viscose, but the affinity for direct dyes such as Pontamine Sky Blue 6BX (C. I. 518) was markedly increased.

#### Example VIII

One-half ( $\frac{1}{2}$ ) part of a 7% solution of a water insoluble room temperature alkali-soluble glycol cellulose in 7% aqueous caustic soda described in Example XXIII were mixed with 99.5 parts of a viscose containing 7% cellulose and 6% sodium hydroxide. The affinity for direct dyes of the product regenerated from the solution was somewhat less than that of Example VII, but was still considerably greater than that of the viscose filaments.

#### Example IX

Twenty-five (25) parts of a 7% solution of a water insoluble glycol cellulose not dissolved by dilute caustic soda at room temperature but dissolved therein by chilling, in 7% aqueous caustic soda prepared as described in Example XXIV, were 75

mixed with 75 parts of a viscose containing 7% cellulose and 6% sodium hydroxide. The mixture was filtered and cast into film in a sodium sulfate-sulfuric acid bath in the way well known in the viscose art. The wet film was almost as strong as that made from viscose.

Films regenerated from this mixture were dyed in the same direct dye bath as filaments of regenerated cellulose prepared from the viscose alone by the same regeneration procedure. The film containing the ether dyed much more deeply than did the regenerated cellulose film.

#### Example X

Twenty-five (25) parts of a 7% solution of a water insoluble glycol cellulose not dissolved by dilute caustic soda at room temperature but dissolved therein by chilling, in 7% aqueous caustic soda prepared as described in Example XXIV, were mixed with 75 parts of a viscose containing 7% cellulose and 6% sodium hydroxide. The viscose-like solution was cast into films in the usual way and was then coated with a lacquer based on ethyl cellulose. The coated film could be immersed in water for several days without the lacquer layer becoming sufficiently loosened to become easily detached by rubbing gently between the fingers.

#### Example XI

One (1) part of a 7% solution of a water insoluble glycol cellulose not dissolved by dilute caustic soda at room temperature but dissolved therein by chilling, in 7% aqueous caustic soda prepared as described in Example XXIV, was mixed with 99 parts of a viscose containing 7% cellulose and 6% sodium hydroxide. The resulting solution mixture was cast into films in the usual way. The films dyed considerably deeper with direct dyes such as Pontamine Sky Blue 6BX (C. I. 518) than did regenerated cellulose films from the same viscose prepared under comparable conditions.

#### Example XII

One (1) part of a 7% solution of a water insoluble glycol cellulose not dissolved by dilute caustic soda at room temperature but dissolved therein by chilling, in 7% aqueous caustic soda prepared as described in Example XXIV, was mixed with 99 parts of a viscose containing 7% cellulose and 6% sodium hydroxide. The resulting viscose-like product was spun into filaments into a bath of the usual composition containing sodium sulfate, sulfuric acid, glucose and zinc sulfate, in the usual manner. The filaments thus obtained showed a markedly greater affinity for direct dyes than did the viscose rayon prepared from the original viscose in the same spinning bath under the same conditions. The dyeing of the cellulose-cellulose ether filaments was unusually level.

#### Example XIII

Twenty-five (25) parts of a 7% solution of water insoluble sodium cellulose glycolate not dissolved by dilute caustic soda solution at room temperature but dissolved therein upon cooling, in 7% sodium hydroxide prepared as described in Example XXV, were mixed with 75 parts of viscose containing 7% cellulose and 6% sodium hydroxide. After thorough mixing, the viscose-like solution was filtered and cast into films. These films after coating with a moisture-proofing composition in accordance with the disclosure in United States Patent No. 1,737,187 gave a product which could be soaked in water at least ten

times as long as films regenerated from the same viscose under the same conditions before the moisture-proofing film could be removed by rubbing gently between the fingers. The cellulose-cellulose ether films exhibited a strong affinity for basic dyes. The wet strength of the films was well within a commercially useful range, although it was somewhat lower than that of regenerated cellulose film made from the same viscose under similar conditions.

Treatment of the cellulose-cellulose ether films with solutions of salts which give precipitates with solutions of water soluble sodium cellulose glycolate, such as potassium aluminum sulfate, resulted in products which were more water repellent than the starting film. The alum treated film burned with considerable difficulty as compared with ordinary regenerated cellulose.

#### Example XIV

Twenty-five (25) parts of a 7% solution of sodium cellulose glycolate not dissolved by dilute caustic soda solution at room temperature but dissolved therein upon cooling, in 7% sodium hydroxide prepared as described in Example XXV, were mixed with 75 parts of viscose containing 7% cellulose and 6% sodium hydroxide. After thorough mixing, the viscose-like solution was filtered and cast into films. These films after coating with a moisture-proofing composition in accordance with the disclosure in United States Patent No. 1,737,187 gave a product which could be soaked in water at least several times as long as films regenerated from the same viscose under the same conditions before the moisture-proofing film could be removed by rubbing gently between the fingers. The cellulose-cellulose ether films were somewhat less resistant to loosening of their moisture-proof coating by water than the product of Example XIII. The dyeing affinity was much the same as the product of Example XIII, but the wet strength was much improved there-over.

Filaments spun from the same viscose-like mixture at low tension possessed a wet strength equal to approximately 80% of that of filaments spun from the same viscose in the same way. In contrast, the filaments spun from a xanthated cellulose glycolic acid containing the same average number of glycolic acid radicals per glucose unit as did the cellulose-cellulose glycolic acid mixture (based on the total number of glucose units in the mixture) possessed a wet strength approximately equal to only 60% of the regenerated cellulose filaments.

#### Example XV

Two (2) parts of a 7% solution of water insoluble sodium cellulose glycolate not dissolved by dilute caustic soda solution at room temperature but dissolved therein upon cooling, in 7% sodium hydroxide prepared as described in Example XXV, were mixed with 98 parts of viscose containing 7% cellulose and 6% sodium hydroxide. After thorough mixing, the viscose-like solution was filtered, and films and filaments prepared therefrom in the usual manner. The regenerated products had an increased affinity for basic dyestuffs such as Du Pont Methyl Violet NE (C. I. 680).

#### Example XVI

Two (2) parts of a 7% solution of a water insoluble sodium cellulose glycolate which is dissolved by dilute caustic soda at room temperature

(prepared according to Example XXVI), in 7% sodium hydroxide, were mixed with 98 parts of a viscose solution containing 7% precipitatable cellulose. The resulting viscose-like body was 5 cast into film being precipitated in a bath composed of 10% sulfuric acid and 20% sodium sulfate and 70% water.

The films were washed and dried in the usual manner. Dye tests comparing these films with 10 films from the same viscose prepared in the same manner showed that with basic dyes such as Du Pont Methyl Violet NE (C. I. 680) the film containing the small amount of cellulose ether dyed approximately 50% stronger. The wet strength 15 of the cellulose-cellulose ether films was very close to that of the regenerated cellulose films.

#### Example XVII

Twenty (20) parts of a 5% solution of a water 20 insoluble room temperature dilute caustic soda soluble methyl cellulose prepared according to Example XXVII in 8% aqueous sodium hydroxide, were mixed with 80 parts of a viscose containing 7% cellulose and 7% sodium hydroxide. 25 The solution was ripened for 40 hours at 25° C. and then cast into films, using a bath containing 12% sulfuric acid, 20% sodium sulfate and 68% water in the usual manner. The resulting films possessed an excellent wet strength and were 30 dyed considerably deeper with substantive dyes than the corresponding regenerated cellulose. The affinity for moisture-proofing lacquer in the presence of water was many times as great as ordinary regenerated cellulose.

35

#### Example XVIII

One-half ( $\frac{1}{2}$ ) part of a 5% solution of a water insoluble room temperature dilute caustic soda soluble methyl cellulose prepared according to 40 Example XXVII in 8% aqueous sodium hydroxide, was mixed with 99.5 parts of a viscose containing 7% cellulose and 7% sodium hydroxide. The solution was ripened for 24 hours at 25° C. and spun into a bath composed of sodium sulfate, glucose, 45 sulfuric acid, zinc sulfate and water, using a series of guide arrangements adapted to give considerable tension on the regenerated filaments during the regeneration step. The modified regenerated cellulose filaments dyed approximately the same 50 with direct dyes as filaments spun from the corresponding unmodified viscose at lower tension.

#### Example XIX

Twenty-five (25) parts of a 7% solution of a 55 water insoluble methyl cellulose not dissolved by dilute caustic soda at room temperature but dissolved therein by chilling to temperatures approximating the freezing point, prepared according to Example XXVIII in 7% aqueous sodium 60 hydroxide, were mixed with 75 parts of viscose containing 7% precipitatable cellulose and 7% sodium hydroxide. The resulting solution was ripened and spun into filaments in the well-known manner. On dyeing with direct dyes such 65 as Pontamine Sky Blue 6BX (C. I. 518) there was obtained a product with a depth of color about twice that obtained from the corresponding viscose rayon.

#### Example XX

70 Twenty-five (25) parts of a 7% solution of a water insoluble methyl cellulose not dissolved by dilute caustic soda at room temperature but dissolved therein by chilling to temperatures approximating the freezing point, prepared accord-

ing to Example XXVIII in 7% aqueous sodium hydroxide, were mixed with 75 parts of viscose containing 7% precipitatable cellulose and 7% sodium hydroxide. Upon regenerating the mixture at a sodium chloride index of 2, films were 5 obtained of excellent wet strength. They showed a greater affinity for direct dyes than the corresponding regenerated cellulose. After drying some of the cellulose-cellulose ether films were 10 coated with a nitrocellulose base moisture-proofing lacquer. It required more than three days soaking in water to loosen the moisture-proof layer sufficiently to enable it to be detached by rubbing gently between the fingers.

Filaments spun from the viscose-like solution 15 possessed a wet strength only slightly inferior to that of yarn spun from unmodified viscose. Filaments spun from a xanthated methyl cellulose containing the same proportion of methyl groups as the viscose-methyl cellulose mixture solution (based upon the sum of the glucose units present in the methyl cellulose and the cellulose) 20 possessed a wet strength of only about 80% of that of the viscose-rayon. Comparable conditions were employed in xanthating the regenerating the 25 methyl cellulose referred to.

#### Example XXI

One (1) part of a 7% solution of a water insoluble methyl cellulose not dissolved by dilute caustic 30 soda at room temperature but dissolved therein by chilling to temperatures approximating the freezing point, prepared according to Example XXVIII in 7% aqueous sodium hydroxide, was mixed with 99 parts of viscose containing 7% 35 precipitatable cellulose and 7% sodium hydroxide. The viscose was ripened and then spun into filaments, using one of the common coagulating baths containing sulfuric acid, glucose, sodium sulfate, and zinc sulfate. The filaments gave a 40 markedly increased affinity for Pontamine Sky Blue 6BX (C. I. 518), a direct dye, when compared with the corresponding viscose-rayon.

#### Example XXII

45 One hundred and sixty (160) parts of sulfite cellulose were steeped in 2000 parts of 18% sodium hydroxide. After one hour at 25° C. the alkali cellulose was pressed to 400 parts and then shredded for two hours at 35° C. It was then 50 placed in a baratte (tumbling device) and provided with a means of vaporizing ethylene oxide into the interior. Eighty-eight (88) parts of ethylene oxide were allowed to vaporize into the apparatus at 20° C. over a period of twelve hours. The resulting product was aged for 24 hours at 25° C. A test sample showed the aged product to be water soluble. An aqueous stock solution containing 6% of the glycol cellulose and 7% sodium hydroxide was then prepared.

#### Example XXIII

55 One hundred and sixty (160) parts of sulfite cellulose were steeped in 2000 parts of 18% caustic soda at 25° C. After one hour the alkali cellulose was pressed to 400 parts and shredded for two hours at 45° C. It was then treated with 22 parts of ethylene oxide at 25° C. for two hours. After ageing for three days at 25° C., it was dissolved at 20° C. in 7% aqueous sodium hydroxide 65 to give a stock solution of 7% glycol cellulose.

#### Example XXIV

70 One hundred (100) parts of sulfite wood pulp were steeped in 1600 parts of 18% caustic for one 75

hour at 25° C. The alkali cellulose was then pressed to 400 parts, shredded for two hours at 30° C., treated with 11 parts of ethylene oxide at 25° C. for two hours and then aged for twenty hours at 30° C. to reduce viscosity. The resulting glycol cellulose was insoluble in dilute caustic soda at room temperature. It was formed into a 7% stock solution in 7% aqueous sodium hydroxide before cooling to -6° C. As soon as the material had again acquired room temperature (25° C.) a perfectly stable solution resulted.

This ether is an example of those low substituted cellulose ethers which are not initially soluble (dissolved by) dilute (6%) aqueous caustic soda at room temperature but which are dissolved therein by cooling to temperatures near the freezing point of the mixture.

#### Example XXV

One hundred and sixty (160) parts of oven dried sulfite pulp were steeped in 1600 parts of 20% caustic for two hours at 25° C. The alkali cellulose was pressed to 400 parts, placed in a shredder with 40 parts of sodium chloroacetate and shredded for three hours. The reaction mixture was then removed from the shredder and aged for 40 hours at 25° C. The resulting cellulose glycolic acid which was not dissolved in dilute caustic soda (4%-10%) solutions at room temperature was made into a 7% solution in 7% sodium hydroxide by cooling a mixture of the cellulose glycolic acid and sodium hydroxide in proper proportions to -8° C.

#### Example XXVI

One hundred and sixty (160) parts of air dried cotton linters of the type used in the manufacture of rayon were steeped in 25% caustic for one hour at 25° C., pressed to 480 parts, and mixed in a Werner-Pfleiderer shredder for three hours at 20° C., with 120 parts of dry sodium chloroacetate. After ageing for sixteen hours the product was dissolved in 7% aqueous caustic soda to form a 7% stock cellulose ether solution. The solution was effected by mixing at 20° C.

#### Example XXVII

One hundred and sixty (160) parts of air dried sulfite cellulose were steeped in 18% caustic for one hour at 25° C. and then pressed to 480 parts. This alkali cellulose was then treated with 134 parts of dimethyl sulfate at room temperature. After shredding for three hours the product was removed and permitted to age for 24 hours at 25° C. It was then water insoluble but dissolved in dilute aqueous caustic soda at room temperature. The product was washed with warm water until free of caustic, after which it was dissolved to give a solution containing 5% cellulose and 8% sodium hydroxide. It was filtered through cotton batting.

#### Example XXVIII

One hundred and sixty (160) parts of sulfite cellulose were steeped in 18% caustic for one hour at 25° C., pressed to 480 parts, mixed in a shredder with 35 parts of dimethyl sulfate at 20° C., removed and aged for 24 hours at 25° C. The product was purified by washing with hot water until free of alkali, then dissolved to give an aqueous solution containing 7% cellulose and 7% sodium hydroxide by cooling to -5° C. Tests showed this methyl cellulose to be insoluble in water and dilute aqueous caustic soda at room temperature but dissolved in dilute aque-

ous caustic soda by chilling to above and near the freezing point. Before the cooling referred to above in the preparation of the solution, the product was essentially undissolved by the caustic soda. After cooling it gave a solution stable at 25° C.

The cellulose xanthate may be made by any of the methods known in the viscose art. It makes little difference what sort of cellulose the viscose is made from, so long as it is one of the types satisfactory for the preparation of viscose suitable for the manufacture of films and filaments by present day commercial practice. A viscose of about 40 poises viscosity in 7% solution in 7% sodium hydroxide at 25° C. is preferred, although other viscosities and concentrations are suitable.

Any cellulose ether which is soluble in alkali may be used to modify the viscose. The invention is most satisfactorily operated with those cellulose ethers which are not dissolved by water or caustic soda at room temperature but which are dissolved in dilute aqueous caustic soda upon cooling to below 0° C. In general, cellulose ethers soluble in caustic alkali and soluble in water, cellulose ethers insoluble in water but dissolved by caustic alkali at room temperature and at low temperatures approximating the freezing point of the mixture, and the cellulose ethers which are not dissolved by water or caustic soda at room temperature but which are dissolved under suitable conditions in dilute aqueous caustic soda chilling to above and near the freezing point, may be used.

Among the caustic alkali soluble ethers suitable for modifying the regenerated cellulose, special mention may be made of methyl cellulose, ethyl cellulose, glycol cellulose, propylene glycol cellulose, isobutylene glycol cellulose, cyclohexene glycol cellulose, glycetyl cellulose, cellulose glycolic acid, and cellulose propionic acid. Mixed cellulose ethers such as methyl cellulose glycolic acid and methyl glycol cellulose, operate satisfactorily, providing the required solubility is present.

In general 25% of any of the alkali soluble ethers is sufficient to give the desired effect. Quantities appreciably greater than 25% confer undesirable properties on the yarn, such as harshness, low wet strength, etc. In most instances lower proportions can be tolerated safely. Ethers soluble in water are ordinarily used in limited amounts because larger quantities tend to lower the wet strength of the product to a degree which is undesirable for many purposes. The cellulose ethers which are dissolved by caustic alkali at room temperature and at low temperatures but which are not dissolved by water, are less prone to cause trouble. The lower substituted ethers, particularly the alkyl celluloses, which are dissolved by dilute aqueous caustic soda at low temperatures approximating the freezing point but are not dissolved thereby at room temperature, are the most satisfactory of all for this purpose, and they constitute a preferred embodiment of the invention.

For most purposes, such as to effect modification of dyeing characteristics, 5% of the alkali soluble ether is a sufficient quantity of modifying agent, and employment of amounts up to 5% is the preferred range. This amount is large enough to give a significant effect, but small enough to leave the physical properties of the modified regenerated products only slightly changed compared with those of regenerated

cellulose alone. For the purposes of dyeing control, the utilization of less than 1% of modifying agent is especially desirable since this gives a marked effect on dyeing characteristics with practically no change in the usual physical characteristics. The products of this invention are so sensitive to dyeing that percentages of cellulose ether as low as 1% and less in the regenerated material in many cases serve to correct variations in production procedures and raw materials.

The effect of the caustic alkali soluble ethers upon the properties of articles regenerated in accordance with this invention such as resistance to changes in size (dimension) with changes in humidity or affinity for moisture-proofing lacquer, is about the same, regardless of the degree of the substitution of the ether. A glycol cellulose soluble in water and present in the viscose in a quantity equal to 15% of the total precipitable matter in the cellulose ether-viscose mixture has about the same effect on the aforementioned resistance to deformation as 15% of a glycol cellulose which is dissolved only by dilute aqueous caustic soda at about the freezing point. The same relationship appears to hold for the other ethers.

The cellulose ethers used in the hereinbefore described processes are (in general) prepared by treating an alkali cellulose with an etherifying agent or any of the other practical cellulose etherification methods. Cellulose glycolic acids whose sodium salts are soluble in water or insoluble in water and dissolved by caustic alkali at room temperature, are well-known, especially in the patent literature. The same is true of methyl cellulose soluble in 6% caustic soda at room temperature but insoluble in water. Cellulose glycolic acids which are not dissolved (in the form of the sodium salt) by caustic soda at room temperature but which are dissolved therein upon cooling to near the freezing point thereof, are described in United States Patent No. 2,060,056. Methyl celluloses which are insoluble in water and caustic soda at room temperature but which dissolve in dilute aqueous caustic soda upon cooling to near the freezing point, are described in United States patent application Serial No. 180,964 filed December 21, 1937. The preparation of such glycol celluloses is described in United States Patent No. 1,941,278.

The viscose-cellulose ether mixture may be made in any desirable or convenient manner. Mention may be made of such procedures as the addition of the cellulose ether to the cellulose xanthate followed by solution of the mixture of the two (accompanied by cooling if necessary), the addition of the undissolved ether to a viscose, and the addition of a solution of the cellulose ether in caustic alkali to the viscose. In some cases it may be desirable to dissolve the cellulose ether in a solution of caustic alkali and then to dissolve the xanthate in the resultant. In general any procedure which results in a homogeneous mixture (solution) of the cellulose xanthate and the cellulose ether is satisfactory. Vigorous agitation is often necessary to accomplish solution, since the salt present in the viscose or cellulose xanthate sometimes exerts a salting-out action on the cellulose ether. This is particularly true when the cellulose ether is of a very low substituted variety. The ethers may be added as solutions of their crude reaction mixtures if found convenient.

The viscose-cellulose ether mixtures are very

much like viscose in their properties so long as the specified limits of quantities of cellulose ether set out above are not exceeded, and their regeneration can be carried out by any of the procedures used in the viscose art. Among the various well-known coagulating baths the following, in addition to those mentioned in the specific examples, are especially suitable:

1. Sulfuric acid (13%) plus sodium sulfate (18%).
2. Sulfuric acid (8%) plus sodium sulfate (26%), plus dextrose (4%).
3. Sulfuric acid (0.5 molar) plus magnesium sulfate (0.1 molar).
4. Sulfuric acid (0.5 molar) plus ammonium sulfate (0.5 molar).
5. Sulfuric acid (0.5 molar) plus sodium sulfate (0.5 molar).

In the spinning of high tenacity yarns, high sulfuric acid concentration baths (above 40%) are particularly applicable.

The regeneration may involve spinning into acid baths of high concentration or into baths provided with special guide arrangements designed and adapted to apply tension to the filaments, as will be clear from the specific examples.

In purifying the regenerated products the usual regenerated cellulose purification methods ordinarily suffice. Where cellulose glycolic acid has been used as the modifying cellulose ether, it is advisable to use neutral or slightly acidic washing and treating media to prevent formation of the corresponding alkali metal salt. Where such a treatment is inadvisable the regenerated product may be given an acid treatment to coagulate (regenerate) the glycolic acid, and the same followed by second washing with water.

Delusterants or other conventional modifying agents may be added to the viscose-cellulose ether mixture.

The dyeing characteristics of the modified rayon of this invention may be controlled by using extremely small quantities of the cellulose ether. As is well-known, variations in the spinning conditions with ordinary viscose gives yarns having different dyeing characteristics. This disadvantage is overcome by the incorporation of a regulated proportion of an alkali soluble cellulose ether in the viscose. Correction of the differences in dye affinity is particularly important in the case of high tenacity rayons which are spun under high tension because they possess a lower affinity for direct dyes than ordinary viscose rayon. The two types of rayon can be given substantially the same affinity for direct dyes simply by including a small proportion of an alkali soluble cellulose ether solution. For example, the incorporation of methyl cellulose in viscose from which high tenacity yarn is spun results in a product having very desirable dyeing characteristics. Likewise, the difference in dyeing characteristics brought about by the use of certain types of cellulose such as cotton linters in making the viscose can be overcome.

The salt forming power of the cellulose glycolic and other oxy-acid ethers of cellulose is of considerable interest because it permits the introduction of many metallic ions into the yarn. For example, treatment of the yarn with copper salts gives a yarn containing copper. Similarly, lead, aluminum, silver, iron and other insoluble salts can be formed. Such products are of especial interest for the preparation of fireproof fabrics, yarns resistant to mildew, etc. This property of salt formation must be taken into con-

sideration since in treatments with soaps, alkaline water, etc., alkali metal salts are formed with a consequent reduction in wet strength.

The films and filaments prepared according to this invention may be used in the same manner as present day films and filaments of regenerated cellulose, with due regard to the superior properties of the products of this invention.

It has been found possible to esterify the free cellulosic hydroxyl groups of the regenerated cellulose of the filaments containing a small proportion of alkali soluble ether much more readily than viscose rayon simply by heating with carboxylic acid anhydrides with or without diluents. 15 Water repellent yarns of excellent appearance may be prepared in this manner. In such esterification processes alkaline or acid catalysts may be used to promote the reaction, and if desired the yarn may be swelled with water or other 20 pretreating agents to assist in the esterification.

As many apparently widely different embodiments of this invention may be made without departing from the spirit and scope thereof, it is to be understood that I do not limit myself to the 25 specific embodiments thereof except as defined in the appended claims.

I claim:

1. A viscose-cellulose ether solution in which not more than 1% of the regeneratable material 30 is a cellulose ether capable of being dissolved in caustic alkali.

2. A modified regenerated cellulose containing up to 5% of an alkali soluble cellulose ether, said product having greater affinity for direct dyes 35 and substantially the same wet strength as unmodified regenerated cellulose.

3. A modified regenerated cellulose containing up to 5% of a water insoluble dilute alkali soluble cellulose ether.

4. A modified regenerated cellulose containing up to 1% of a cellulose ether dissolved by dilute aqueous caustic soda at low temperatures approximating the freezing point but not dissolved thereby at room temperature, said product having 45 greater affinity for direct dyes and substantially the same wet strength as unmodified regenerated cellulose.

5. A viscose-cellulose ether solution in which not more than 5% of the regeneratable material

is a cellulose ether capable of being dissolved in caustic alkali.

6. A modified regenerated cellulose containing up to 1% of an alkali soluble cellulose ether, said product having greater affinity for direct dyes 5 and substantially the same wet strength as unmodified regenerated cellulose and said product having been prepared by regenerating a cellulose xanthate-alkali soluble cellulose ether solution.

7. A modified regenerated cellulose containing 10 up to 5% of a water insoluble dilute alkali soluble cellulose glycolic acid ether, said product having greater affinity for basic dyes and substantially the same wet strength as unmodified regenerated cellulose and said product having 15 been prepared by regenerating a cellulose xanthate-alkali soluble cellulose ether solution.

8. A modified regenerated cellulose containing up to 1% of a glycol cellulose ether dissolved by dilute aqueous caustic soda at low temperatures 20 approximating the freezing point but not dissolved thereby at room temperature, having greater affinity for direct dyes and substantially the same wet strength as unmodified regenerated cellulose and said product having been prepared 25 by regenerating a cellulose xanthate-alkali soluble cellulose ether solution.

9. A modified regenerated cellulose containing up to 5% of a low alkyl (methyl or ethyl) cellulose ether, the said cellulose ether not being dissolved by water or aqueous caustic soda at room 30 temperature, but which is dissolved in dilute aqueous caustic soda upon chilling to above and near the freezing point, said product having greater affinity for direct dyes and substantially 35 the same wet strength as unmodified regenerated cellulose.

10. A modified regenerated cellulose containing up to 5% of a low substituted glycol cellulose, said glycol cellulose being insoluble in water and 40 soluble in aqueous caustic soda, said product having greater affinity for direct dyes and substantially the same wet strength as unmodified regenerated cellulose and said modified regenerated cellulose having been prepared by regenerating a 45 cellulose xanthate-alkali soluble glycol cellulose ether solution.

ROBERT W. MAXWELL.

CERTIFICATE OF CORRECTION.

Patent No. 2,162,460.

June 13, 1939.

ROBERT W. MAXWELL.

It is hereby certified that error appears in the printed specification of the above numbered patent requiring correction as follows: Page 5, second column, line 33, before the word "chilling" insert upon; line 41, for "gycolic" read glycolic; and that the said Letters Patent should be read with this correction therein that the same may conform to the record of the case in the Patent Office.

Signed and sealed this 1st day of August, A. D. 1939.

(Seal)

Henry Van Arsdale,  
Acting Commissioner of Patents.

sideration since in treatments with soaps, alkaline water, etc., alkali metal salts are formed with a consequent reduction in wet strength.

The films and filaments prepared according to this invention may be used in the same manner as present day films and filaments of regenerated cellulose, with due regard to the superior properties of the products of this invention.

It has been found possible to esterify the free cellulosic hydroxyl groups of the regenerated cellulose of the filaments containing a small proportion of alkali soluble ether much more readily than viscose rayon simply by heating with carboxylic acid anhydrides with or without diluents. 15 Water repellent yarns of excellent appearance may be prepared in this manner. In such esterification processes alkaline or acid catalysts may be used to promote the reaction, and if desired the yarn may be swelled with water or other 20 pretreating agents to assist in the esterification.

As many apparently widely different embodiments of this invention may be made without departing from the spirit and scope thereof, it is to be understood that I do not limit myself to the 25 specific embodiments thereof except as defined in the appended claims.

I claim:

1. A viscose-cellulose ether solution in which not more than 1% of the regeneratable material 30 is a cellulose ether capable of being dissolved in caustic alkali.

2. A modified regenerated cellulose containing up to 5% of an alkali soluble cellulose ether, said product having greater affinity for direct dyes 35 and substantially the same wet strength as unmodified regenerated cellulose.

3. A modified regenerated cellulose containing up to 5% of a water insoluble dilute alkali soluble cellulose ether.

4. A modified regenerated cellulose containing up to 1% of a cellulose ether dissolved by dilute aqueous caustic soda at low temperatures approximating the freezing point but not dissolved thereby at room temperature, said product having 45 greater affinity for direct dyes and substantially the same wet strength as unmodified regenerated cellulose.

5. A viscose-cellulose ether solution in which not more than 5% of the regeneratable material

is a cellulose ether capable of being dissolved in caustic alkali.

6. A modified regenerated cellulose containing up to 1% of an alkali soluble cellulose ether, said product having greater affinity for direct dyes 5 and substantially the same wet strength as unmodified regenerated cellulose and said product having been prepared by regenerating a cellulose xanthate-alkali soluble cellulose ether solution.

7. A modified regenerated cellulose containing 10 up to 5% of a water insoluble dilute alkali soluble cellulose glycolic acid ether, said product having greater affinity for basic dyes and substantially the same wet strength as unmodified regenerated cellulose and said product having 15 been prepared by regenerating a cellulose xanthate-alkali soluble cellulose ether solution.

8. A modified regenerated cellulose containing up to 1% of a glycol cellulose ether dissolved by dilute aqueous caustic soda at low temperatures 20 approximating the freezing point but not dissolved thereby at room temperature, having greater affinity for direct dyes and substantially the same wet strength as unmodified regenerated cellulose and said product having been prepared 25 by regenerating a cellulose xanthate-alkali soluble cellulose ether solution.

9. A modified regenerated cellulose containing up to 5% of a low alkyl (methyl or ethyl) cellulose ether, the said cellulose ether not being dissolved by water or aqueous caustic soda at room 30 temperature, but which is dissolved in dilute aqueous caustic soda upon chilling to above and near the freezing point, said product having greater affinity for direct dyes and substantially 35 the same wet strength as unmodified regenerated cellulose.

10. A modified regenerated cellulose containing up to 5% of a low substituted glycol cellulose, said glycol cellulose being insoluble in water and 40 soluble in aqueous caustic soda, said product having greater affinity for direct dyes and substantially the same wet strength as unmodified regenerated cellulose and said modified regenerated cellulose having been prepared by regenerating a 45 cellulose xanthate-alkali soluble glycol cellulose ether solution.

ROBERT W. MAXWELL.

CERTIFICATE OF CORRECTION.

Patent No. 2,162,460.

June 13, 1939.

ROBERT W. MAXWELL.

It is hereby certified that error appears in the printed specification of the above numbered patent requiring correction as follows: Page 5, second column, line 33, before the word "chilling" insert upon; line 41, for "gycolic" read glycolic; and that the said Letters Patent should be read with this correction therein that the same may conform to the record of the case in the Patent Office.

Signed and sealed this 1st day of August, A. D. 1939.

(Seal)

Henry Van Arsdale,  
Acting Commissioner of Patents.